

July 9, 1929.

P. J. PEYRACHON

1,720,055

APPARATUS FOR MANUFACTURING IRON AND STEEL

Filed May 2, 1927

2 Sheets-Sheet 1



Pierre Joseph Peyrachon

INVENTOR;

By *John M. Peacock*  
his Attorney.

July 9, 1929.

P. J. PEYRACHON

1,720,055

APPARATUS FOR MANUFACTURING IRON AND STEEL

Filed May 2, 1927

2 Sheets-Sheet 2

Fig. 3.



Fig. 5.



Fig. 4



Fig. 6.



Pierre Joseph Peyrachon  
INVENTOR;  
By *Ottolunk*  
his Attorney

## UNITED STATES PATENT OFFICE.

PIERRE JOSEPH PEYRACHON, OF LA FELGUERA, SPAIN.

## APPARATUS FOR MANUFACTURING IRON AND STEEL.

Application filed May 2, 1927, Serial No. 188,095, and in France July 13, 1926.

One of the chief disadvantages which has, up to the present time, prevented rotary furnaces from being extensively used in the modern manufacturing of iron is the great wear and tear on the lining of the lower section of the furnace, due to the high temperature to which this part of the apparatus is subjected and to the precarious cooling means employed.

10 The use of pulverized carbon in the manufacture of open hearth steel, such as in the Siemens-Martin process, has likewise not come into extensive use because of the rapid filling up of the regenerating chambers by 15 the fine dust raised by the cinder of the pulverized carbon.

The object of this invention is, in general, to overcome the disadvantages above enumerated.

20 To this end I provide the lining of my rotary furnace with a protecting screen, directly in contact with the rising flames of the furnace and extending around the greater portion of its circumference. The invention

25 is equally applicable to both the stationary type and tilting type of furnace. Furthermore to further assure the cooling of the lining, a movable hollow ring kept entirely filled with water is provided. The rising

30 gases are arranged to pass out of the upper part of the foundation which receives the lower section of the rotary furnace thus preventing the flames from contacting with the lining of the lower section of the furnace.

35 The open hearth furnace I use may constitute but a single chamber for receiving the metal whether it be of the stationary type such as the Martin furnace or of the movable type such as the Wellmann furnace. I provide a dust chamber in communication with a rotary carburizing furnace connected to a gas producing apparatus which burns all traces of combustible material.

40 My furnace is capable of producing pig-iron or a less carbonized metal without silicon or sulfur, which metal is very liquid and becomes very hot.

The annexed drawing taken with the specification, illustrates by way of example, an apparatus constructed after the principle of my invention. In the drawing,

45 Fig. 1 is a view in elevation of the assembled apparatus, parts being shown in section;

50 Fig. 2 is a plan view of the apparatus;

Fig. 3 is a section along line 3—3 of Fig. 2; Fig. 4 is a section along line 4—4 of Fig. 3; Fig. 5 is a section of parts illustrated in Fig. 1 but drawn to a larger scale to more clearly illustrate the invention, and Fig. 6 is a detail of certain parts of the apparatus.

55 Referring to the drawing, A represents a cylindrical rotary reducing furnace, slightly inclined from the horizontal. This furnace may be of any well known type of rotary furnace and is furnished with an interior refractory lining carried by the metallic casing of the furnace and extending the full length of the furnace as is well known in the art.

60 Fixed to the lower extremity of furnace A is a ring A<sup>1</sup> of cast iron or steel and which may be cylindrical but as here shown takes the form of a truncated cone. This ring is arranged to have water circulated through it, cold water being admitted at the lowest portion and the hot water being drawn off at the top.

65 Ring A<sup>1</sup> (Fig. 6) is closed by means of a cover a in the form of an annulus, cut from sheet iron or steel and bearing against appropriate annular flanges c, c, carried by ring A<sup>1</sup>. Member a is held in place by means of springs d placed at intervals along its circumference. Said springs are provided with rollers v, which bear against a flange b fixed to the casing of furnace A and rotatable therewith, at one end and bear against cover a at the other end.

70 Ring A<sup>1</sup> projects into a metallic housing B which is lined with a refractory material. Within this lining are formed two vertical channels f, f, symmetrically spaced with respect to the vertical axis of housing B and two horizontal channels connecting said vertical channels with the upper portion of housing B.

75 A masonry arch g of refractory material is provided on the interior of member B and serves as a protecting screen for the lower end of furnace A. This arch may, if necessary, be cooled interiorly by a water jacket.

80 On the lower portion of housing B is formed a base which is cooled by a water spray, and opens into the smelting furnace C. The rotary furnace A is placed into communication with furnace C by means of the opening h piercing the arch of the latter.

85 The smelting furnace C is of masonry and

consists of a suitable refractory material held together by steel or iron plates. The upper portion of the furnace takes the shape of an inverted truncated cone and the lower portion that of a cylinder in which are lodged a plurality of interiorly cooled tuyères *i*. Said cylindrical portion is lined with a refractory material and constitutes the crucible of the furnace.

10 On the periphery of the crucible near the lower part are disposed a number of openings *o* which connect with the interior of the furnace. Into each of these openings is inserted a carbon electrode *a*. The crucible is 15 further provided with a tap *p* for drawing off the metal and a tap *q* for drawing off the slag. The hearth of the furnace is of masonry and of a refractory material.

D is a rotary carburizing furnace comprising 20 an inclined cylinder furnished with a refractory lining similar to but shorter than furnace A. The extremities of the cylinder are provided with rings similar to ring A<sup>1</sup> of furnace A. The extremities of furnace D are housed in casings F, F<sup>1</sup>, lined with a refractory material.

Housing F is furnished with an opening and a damper which connects with a pipe G leading to housing B. Housing F<sup>1</sup> likewise 30 is connected to an open hearth furnace L by means of pipe K which communicates with opening *t* in said housing.

H represents any suitable gas producing apparatus which is provided with a pipe *u* for injecting air and steam.

The open hearth furnace L comprises a melting chamber, one end of which connects with a dust chamber M while the other end is closed by a removable shield N which carries 40 the cooled tuyères *j*.

W is a tap for drawing off the metal and Z is a funnel like spout through which the furnace is charged with the molten metal from C.

45 A tuyère *k* is placed on housing F<sup>1</sup> and a tuyère *l* is placed on housing B.

Helical screw conveyors *m* and *n* carry the materials to reducing furnace A and the combustible to the carburizing furnace D respectively.

The upper extremity of reducing furnace A is provided with a dust chamber O in which any large dust particles carried along by the gas coming from A are caught. The 55 gas is then led to gas washers through pipe *x* in the usual manner. The lower portion of chamber O is closed by a water seal P.

The function of the apparatus is as follows:

60 Once the apparatus is started, ore mixed with the proper quantity of carbon is introduced into the rotary furnace A by means of conveyor *m*. The carbon may be in the form of lignite coal, peat, charcoal or wood. A 65 small amount of flux is added, also through

conveyor *m* to give the proper consistency to the molten mass.

The materials introduced by the conveyor *m* become heated and the ore is reduced during their travel through furnace A. 70 They attain a temperature of from 1,000 to 1,100 degrees centigrade upon leaving furnace A.

The molten mass then tumbles to the bottom of funnel-shaped casing B and thence 75 into the reducing furnace C through opening *h*. The molten mass accumulates in the crucible of furnace C, where it is subjected to heat by means of an electric current brought in by carbons *a*. The metal then 80 separates from the slag and descends to the bottom of the crucible where it is drawn off periodically through tap *p*, while the slag which forms above is drawn off through tap *q*. The apparatus thus far described 85 produces iron.

In order to obtain steel it is only necessary to add through opening *y* provided in housing B for that purpose, a mixture of ore and limestone for the purpose of oxidizing the 90 excess carbon as well as the silicium coming from the silica of the gangue which will be reduced by the carbon at the moment fusion of the mixture takes place.

The quantity of ore to be added may be 95 determined from the results of an analysis of a sample taken from the material issuing from furnace A. The introduction of the ore may be through the medium of an automatic apparatus if desired. The apparatus thus far described produces soft steel nearly free from silicium and of which the carbon content varies from 0.5% to 2%.

The metal on leaving furnace C may now 100 be conveyed to open hearth furnace L into which it is introduced through the opening Z, where a further refining takes place and the necessary additions are made for obtaining the quality of steel desired. Through the charging doors of furnace L, scrap iron and 105 other waste metal may be introduced as well as the refining materials.

When the refining is completed, the metal is drawn off into ingot moulds which are 110 placed in a pit R, through tap *w*.

A liquid, solid or gaseous combustible is 115 mixed with hot air and introduced into furnace L by means of tuyères *j*. The mixture burns in the melting chamber of said furnace forming carbonic acid gas exclusively 120 and gives to the furnace the necessary heat to accomplish the refining operation. The gases of combustion are led from the melting chamber into the dust chamber and thence into pipe K where they enter the lower extremity of furnace D through housing F<sup>1</sup>.

In furnace D, the solid combustible material is introduced in its upper end by means of conveyor *n*. Under the influence of the 130 heat content of the gases of combustion and

their high temperature, the carbonic acid which they contain is reduced to carbonic oxide. The carbonic oxide and carbonic acid content is at least 9 parts by weight when the 5 gas leaves furnace D.

The tuyère situated on housing F<sup>1</sup> is used to inject a mixture of a solid, liquid or gaseous combustible and hot air carrying sufficient heat to effect the reduction of the carbonic 10 acid thus maintaining the temperature of the gases between 1250 and 1300 degrees centigrade at the point of leaving the furnace.

The gases leaving furnace D are conducted by the pipes G to housing B where they enter 15 at a temperature from 1150 to 1250 degrees centigrade. The gases here mix with those issuing from furnace C through channels f, pass into the furnace A and there supply the necessary amount of heat for producing 20 the required temperature to bring about the chemical actions necessary for reducing the mass of ore contained in furnace A.

The gases on leaving furnace A pass into the dust chamber O and from there are led 25 to gas washers by means of pipe line x and are finally utilized in regenerators or other apparatus for the utilization of their energy content.

The combustible contained in furnace D 30 burns when it contacts with the hot gases circulating therein. At the lower extremity of furnace D the residues of combustion enter the housing F<sup>1</sup> and pass into the gas producer H by opening S where the residue of combustion accumulates. This residue which consists of a mixture of cinders and coke is subjected to a current of air and steam issuing 35 from pipe u. This air becomes heated in contacting the incandescent mass and burns all traces of coke. The cold cinders are drawn 40 from the bottom of the apparatus H whenever necessary.

The tuyère l situated on the front part of housing B may be used to inject either hot 45 air or a mixture of hot air and a combustible for raising the temperature of furnace A at will.

The tuyères i situated on the periphery of the cylindrical part of furnace C are employed at the time of starting the apparatus. 50 They furnish air to the combustible supplied to furnace C. During the functioning of the apparatus they may be used to supply gas from chamber O to the unmelted mass coming 55 from B. This gas contains a certain amount of carbonic acid which reduces the excess carbon content of the mass and at the same time raises its temperature and carries the surplus heat of C to furnace A.

60 It is evident that many modifications might

be made without departing from the scope of the invention as set forth in the appended claims. For example, open hearth furnace L might be replaced by an electric refining furnace. In this event furnace L could supply 65 its gases directly by eliminating pipe K and utilizing tuyère k to supply continuously a mixture of hot air and combustible material. The apparatus otherwise would function as previously described. 70

The advantages derived from my invention may be summed up as follows:

The reduction to a minimum of the amount of solid combustible necessary to mix with the ore and consequently a minimum of slag 75 and sulphur present in the molten contents of the furnace.

The utilization of half burned cinders for heating purposes as well as the burning of all sorts of combustible waste material in the 80 carbureting furnace down to the last particle of combustible matter.

The employment of solid pulverized combustible materials in the open hearth furnace. 85

The obtaining of cast iron or a less carbonized metal at will in the smelting furnace, and

The utilization of the waste gases escaping 90 from the open hearth furnace.

Having described my invention, what I claim is:

1. In ore reducing apparatus, the combination of a smelting furnace, a housing superimposed thereon, said housing being interiorly of refractory material with intercommunicating vertical and horizontal channels within said refractory material, a rotary reducing furnace having one of its ends opening into said housing and a refractory 95 flame baffle within the housing adjacent said end of the rotary reducing furnace.

2. In ore reducing apparatus, the combination of a smelting furnace, a housing superimposed thereon, said housing being interiorly of refractory material, a rotary reducing furnace having one of its ends opening into said housing, a water cooled casing about the said end of the rotary reducing furnace, a refractory flame baffle within the housing 100 adjacent said end of the rotary reducing furnace, the refractory material of the housing having interior intercommunicating channels to guide the gases arising from the smelting furnace out of the path of material issuing 110 from the rotary reducing furnace.

Signed at Bilbao, Spain, in the Province of Viscaya and State of Spain, this 11th day of April, A. D. 1927.

PIERRE JOSEPH PEYRACHON.